



US007833953B2

(12) **United States Patent**  
**Devlin et al.**

(10) **Patent No.:** **US 7,833,953 B2**  
(45) **Date of Patent:** **\*Nov. 16, 2010**

(54) **LUBRICANT COMPOSITION**(75) Inventors: **Mark T. Devlin**, Richmond, VA (US);  
**Tze-chi Jao**, Glen Allen, VA (US)(73) Assignee: **Afton Chemical Corporation**,  
Richmond, VA (US)(\* ) Notice: Subject to any disclaimer, the term of this  
patent is extended or adjusted under 35  
U.S.C. 154(b) by 378 days.This patent is subject to a terminal dis-  
claimer.(21) Appl. No.: **11/467,695**(22) Filed: **Aug. 28, 2006**(65) **Prior Publication Data**

US 2008/0051305 A1 Feb. 28, 2008

(51) **Int. Cl.****C10L 1/22** (2006.01)**C10G 71/00** (2006.01)(52) U.S. Cl. .... **508/192**; 208/18; 208/19(58) **Field of Classification Search** .... **508/192**;  
**208/18, 19**

See application file for complete search history.

(56) **References Cited**

## U.S. PATENT DOCUMENTS

|             |         |                    |
|-------------|---------|--------------------|
| 2,063,629 A | 12/1936 | Salzberg et al.    |
| 2,224,695 A | 12/1940 | Prutton            |
| 2,284,409 A | 5/1942  | Erath              |
| 2,284,410 A | 5/1942  | Farmer             |
| 2,447,288 A | 8/1948  | Smith et al.       |
| 2,459,112 A | 1/1949  | Oberright          |
| 2,616,905 A | 11/1952 | Asseff et al.      |
| 2,945,749 A | 7/1960  | Andress, Jr.       |
| 2,962,442 A | 11/1960 | Andress, Jr.       |
| 2,984,550 A | 5/1961  | Chamot             |
| 3,036,003 A | 5/1962  | Dolton             |
| 3,087,936 A | 4/1963  | Le Suer            |
| 3,163,603 A | 12/1964 | Le Suer            |
| 3,166,516 A | 1/1965  | Kirkpatrick et al. |
| 3,172,892 A | 3/1965  | Le Suer et al.     |
| 3,184,474 A | 5/1965  | Catto et al.       |
| 3,202,678 A | 8/1965  | Stuart et al.      |
| 3,215,707 A | 11/1965 | Rense              |
| 3,216,936 A | 11/1965 | Le Suer            |
| 3,219,666 A | 11/1965 | Norman et al.      |
| 3,236,770 A | 2/1966  | Matson et al.      |
| 3,254,025 A | 5/1966  | Le Suer            |
| 3,271,310 A | 9/1966  | Le Suer            |
| 3,272,746 A | 9/1966  | Le Suer et al.     |
| 3,275,554 A | 9/1966  | Wagenaar           |
| 3,281,357 A | 10/1966 | Vogel              |
| 3,281,428 A | 10/1966 | Le Suer            |
| 3,282,955 A | 11/1966 | Le Suer            |
| 3,306,908 A | 2/1967  | Le Suer            |
| 3,311,558 A | 3/1967  | Prizer et al.      |
| 3,316,177 A | 4/1967  | Dorer              |
| 3,329,658 A | 7/1967  | Fields             |
| 3,331,776 A | 7/1967  | Krukzienier        |
| 3,338,832 A | 8/1967  | Le Suer            |

|             |         |                      |
|-------------|---------|----------------------|
| 3,340,281 A | 9/1967  | Brannen              |
| 3,341,542 A | 9/1967  | Le Suer et al.       |
| 3,344,069 A | 9/1967  | Stuebe               |
| 3,346,493 A | 10/1967 | Le Suer              |
| 3,351,552 A | 11/1967 | Le Suer              |
| 3,355,270 A | 11/1967 | Amick et al.         |
| 3,356,702 A | 12/1967 | Farmer et al.        |
| 3,368,972 A | 2/1968  | Otto                 |
| 3,381,022 A | 4/1968  | Le Suer              |
| RE26,433 E  | 8/1968  | Le Suer              |
| 3,399,141 A | 8/1968  | Clemens              |
| 3,413,347 A | 11/1968 | Worrel               |
| 3,415,750 A | 12/1968 | Anzenberger          |
| 3,433,744 A | 3/1969  | Le Suer              |
| 3,438,757 A | 4/1969  | Honnen et al.        |
| 3,442,808 A | 5/1969  | Traise et al.        |
| 3,444,170 A | 5/1969  | Norman et al.        |
| 3,448,047 A | 6/1969  | Traise et al.        |
| 3,448,048 A | 6/1969  | Le Suer et al.       |
| 3,448,049 A | 6/1969  | Preuss et al.        |
| 3,449,250 A | 6/1969  | Fields               |
| 3,451,933 A | 6/1969  | Leister              |
| 3,454,497 A | 7/1969  | Wittner              |
| 3,454,555 A | 7/1969  | van der Voort et al. |
| 3,454,607 A | 7/1969  | Le Suer et al.       |
| 3,459,661 A | 8/1969  | Schlobohm            |
| 3,461,172 A | 8/1969  | Previc               |
| 3,467,668 A | 9/1969  | Gruber et al.        |
| 3,493,520 A | 2/1970  | Verdol et al.        |

(Continued)

## FOREIGN PATENT DOCUMENTS

|    |              |         |
|----|--------------|---------|
| EP | 1136496 A1   | 9/2001  |
| EP | 1136497 A1   | 9/2001  |
| EP | 1 167 497 A2 | 1/2002  |
| EP | 1 364 955 A1 | 11/2003 |
| EP | 1 657 293 A2 | 5/2006  |
| WO | WO 87/07638  | 12/1987 |

## OTHER PUBLICATIONS

M.T. Devlin, et al., "Effect of Detailed Base Oil Structure on Oxidation Performance of Automatic Transmission Fluids," Proceedings of WTC 2005, Sep. 12-16, 2005, pp. 1-2.

Analytical Chemistry, 64:2227 (1992).

M. T. Devlin, T. Hammock, and T-C. Jao, "Effect of Mechanical Shear on the Thin Film Properties of Base Oil-Polymer Mixtures", Lubrication Science vol. 14 (2), 2002.

D. Dawson, et al., "Lubrication at the Frontier: The Role of the Interface and Surface Layers in the Thin Film and Boundary Regime," Elsevier Science B.V., 1999, p. 769-766.

(Continued)

Primary Examiner—Walter D Griffin  
Assistant Examiner—Frank C Campanell(57) **ABSTRACT**

A lubricant composition comprising a dispersant and a base oil comprising more than about 1.6% by weight of tetracycloparaffins is disclosed. Methods of making and using the lubricant composition are also disclosed.

**18 Claims, No Drawings**

## U.S. PATENT DOCUMENTS

|             |         |                   |                   |          |                               |
|-------------|---------|-------------------|-------------------|----------|-------------------------------|
| 3,501,405 A | 3/1970  | Willette          | 4,173,540 A       | 11/1979  | Lonstrup et al.               |
| 3,509,051 A | 4/1970  | Farmer et al.     | 4,178,258 A       | 12/1979  | Papay et al.                  |
| 3,519,565 A | 7/1970  | Coleman           | 4,234,435 A       | 11/1980  | Meinhardt et al.              |
| 3,522,179 A | 7/1970  | Le Suer           | 4,259,195 A       | 3/1981   | King et al.                   |
| 3,533,945 A | 10/1970 | Vogel             | 4,261,843 A       | 4/1981   | King et al.                   |
| 3,539,633 A | 11/1970 | Piasiek et al.    | 4,263,152 A       | 4/1981   | King et al.                   |
| 3,541,012 A | 11/1970 | Stuebe            | 4,265,773 A       | 5/1981   | de Vries et al.               |
| 3,542,680 A | 11/1970 | Le Suer           | 4,266,945 A       | 5/1981   | Karn                          |
| 3,543,678 A | 12/1970 | Hobbs, Jr.        | 4,272,387 A       | 6/1981   | King et al.                   |
| 3,558,743 A | 1/1971  | Verdol et al.     | 4,283,295 A       | 8/1981   | de Vries et al.               |
| 3,565,804 A | 2/1971  | Honnen et al.     | 4,285,822 A       | 8/1981   | de Vries et al.               |
| 3,567,637 A | 3/1971  | Sabol             | 4,354,950 A       | 10/1982  | Hammond et al.                |
| 3,574,101 A | 4/1971  | Murphy            | 4,362,633 A       | 12/1982  | Spence et al.                 |
| 3,576,743 A | 4/1971  | Widmer et al.     | 4,369,119 A       | 1/1983   | de Vries et al.               |
| 3,586,629 A | 6/1971  | Otto et al.       | 4,395,343 A       | 7/1983   | de Vries et al.               |
| 3,591,598 A | 7/1971  | Traise et al.     | 4,402,840 A       | 9/1983   | de Vries et al.               |
| 3,600,372 A | 8/1971  | Udelhofen et al.  | 4,431,552 A       | 2/1984   | Salentine                     |
| 3,630,904 A | 12/1971 | Musser et al.     | 4,455,243 A       | 6/1984   | Liston                        |
| 3,632,510 A | 1/1972  | Le Suer           | 4,466,901 A       | 8/1984   | Hunt et al.                   |
| 3,632,511 A | 1/1972  | Liao              | 4,485,023 A       | 11/1984  | Serres et al.                 |
| 3,634,515 A | 1/1972  | Piasiek et al.    | 4,652,387 A       | 3/1987   | Andress, Jr. et al.           |
| 3,649,229 A | 3/1972  | Otto              | 4,692,256 A       | 9/1987   | Umemura et al.                |
| 3,658,836 A | 4/1972  | Vineyard          | 4,765,918 A       | 8/1988   | Love et al.                   |
| 3,666,730 A | 5/1972  | Coleman           | 4,863,623 A       | 9/1989   | Nalesnik                      |
| 3,687,849 A | 8/1972  | Abbott            | 4,889,647 A       | 12/1989  | Rowan et al.                  |
| 3,697,428 A | 10/1972 | Meinhardt et al.  | 4,966,719 A       | 10/1990  | Coyle et al.                  |
| 3,697,574 A | 10/1972 | Piasiek et al.    | 4,978,464 A       | 12/1990  | Coyle et al.                  |
| 3,702,300 A | 11/1972 | Coleman           | 4,990,271 A       | 2/1991   | Franis                        |
| 3,703,536 A | 11/1972 | Piasiek et al.    | 4,995,996 A       | 2/1991   | Coyle et al.                  |
| 3,704,308 A | 11/1972 | Piasiek et al.    | 5,075,383 A       | 12/1991  | Migdal et al.                 |
| 3,718,663 A | 2/1973  | Piasiek et al.    | 5,137,647 A       | 8/1992   | Karol                         |
| 3,725,277 A | 4/1973  | Worrel            | 5,137,980 A       | 8/1992   | DeGonia et al.                |
| 3,725,441 A | 4/1973  | Murphy            | 5,139,688 A       | 8/1992   | Nalesnik                      |
| 3,725,480 A | 4/1973  | Traise et al.     | 5,230,834 A       | * 7/1993 | Gutierrez et al. .... 508/236 |
| 3,726,882 A | 4/1973  | Traise et al.     | 5,266,223 A       | 11/1993  | Song et al.                   |
| 3,736,357 A | 5/1973  | Piasiek et al.    | 5,350,532 A       | 9/1994   | Song et al.                   |
| 3,751,365 A | 8/1973  | Piasiek et al.    | 5,354,484 A       | 10/1994  | Schwind et al.                |
| 3,756,953 A | 9/1973  | Piasiek et al.    | 5,356,999 A       | 10/1994  | Kapuscinski et al.            |
| 3,793,202 A | 2/1974  | Piasiek et al.    | 5,372,735 A       | 12/1994  | Ohtani et al.                 |
| 3,798,165 A | 3/1974  | Piasiek et al.    | 5,374,364 A       | 12/1994  | Kapuscinski et al.            |
| 3,798,247 A | 3/1974  | Piasiek et al.    | 5,412,130 A       | 5/1995   | Karol                         |
| 3,803,039 A | 4/1974  | Piasiek et al.    | 5,424,366 A       | 6/1995   | Kapuscinski et al.            |
| 3,804,763 A | 4/1974  | Meinhardt         | 5,435,926 A       | 7/1995   | Gutierrez et al.              |
| 3,836,471 A | 9/1974  | Miller            | 5,441,656 A       | 8/1995   | Ohtani et al.                 |
| 3,862,981 A | 1/1975  | Demoures et al.   | 5,634,951 A       | 6/1997   | Colucci et al.                |
| 3,872,019 A | 3/1975  | Culbertson et al. | 5,725,612 A       | 3/1998   | Malfer et al.                 |
| 3,904,595 A | 9/1975  | Plonsker et al.   | 5,763,372 A       | 6/1998   | Tersigni et al.               |
| 3,936,480 A | 2/1976  | Demoures et al.   | 5,789,353 A       | 8/1998   | Scattergood                   |
| 3,948,800 A | 4/1976  | Meinhardt         | 6,103,674 A       | 8/2000   | Nalesnik et al.               |
| 3,950,341 A | 4/1976  | Okamoto et al.    | 6,107,257 A       | 8/2000   | Valcho et al.                 |
| 3,957,746 A | 5/1976  | Malec             | 6,107,258 A       | 8/2000   | Esche, Jr. et al.             |
| 3,957,854 A | 5/1976  | Miller            | 6,117,825 A       | 9/2000   | Liu et al.                    |
| 3,957,855 A | 5/1976  | Miller            | 6,117,826 A       | 9/2000   | Baranski et al.               |
| 3,980,569 A | 9/1976  | Pindar et al.     | 6,232,276 B1      | 5/2001   | Stiefel et al.                |
| 3,984,448 A | 10/1976 | Lippsmeier        | 2005/0250655 A1 * | 11/2005  | Adams et al. .... 508/287     |
| 3,985,802 A | 10/1976 | Piasiek et al.    | 2006/0094607 A1 * | 5/2006   | Devlin et al. .... 508/563    |
| 3,991,098 A | 11/1976 | Okamoto           |                   |          |                               |
| 4,006,089 A | 2/1977  | Chibnik           |                   |          |                               |
| 4,011,380 A | 3/1977  | West et al.       |                   |          |                               |
| 4,025,451 A | 5/1977  | Plonsker et al.   |                   |          |                               |
| 4,058,468 A | 11/1977 | Malec             |                   |          |                               |
| 4,071,548 A | 1/1978  | Okamoto           |                   |          |                               |
| 4,083,699 A | 4/1978  | Chibnik           |                   |          |                               |
| 4,090,854 A | 5/1978  | Davis             |                   |          |                               |
| 4,098,705 A | 7/1978  | Sakurai et al.    |                   |          |                               |
| 4,164,473 A | 8/1979  | Coupland et al.   |                   |          |                               |

## OTHER PUBLICATIONS

R.C. Castle, et al., "The Behavior of Friction Modifiers Under Boundary and Mixed EHD Conditions," SAE 961142, pp. 1-4.

Lisa Taylor, et al. "Film-Forming Properties of Zinc-Based and Ashless Antiwear Additives," International Spring Fuels & Lubricants, Paris, France, Jun. 19-22, 2000, pp. 1-11.

M.T. Devlin, et al. "Improved Understanding of Axle Oil Rheology Effects on Torque Transfer Efficiency and Axle Oil Operating Temperature," SAE 2003-01-1972, 2003, pp. 1-10.

\* cited by examiner

## 1

## LUBRICANT COMPOSITION

## DESCRIPTION OF THE DISCLOSURE

## 1. Field of the Disclosure

The present disclosure relates to a lubricating composition comprising a dispersant and a base oil comprising more than about 1.6% by weight of tetracycloparaffins.

## 2. Background of the Disclosure

In recent years there has been growing concern to produce transmission fluids that can increase torque transferred through a transmission and prevent shudder. Moreover, modern transmission fluid specifications require lubricants to demonstrate high torque capacity and shudder prevention properties. The frictional characteristics of thin lubricant films are known to affect torque capacity and shudder prevention properties of oils.

Thin-film friction is the friction generated from fluid, such as a lubricant, pushing between two surfaces, wherein the distance between the two surfaces is very narrow. It is known that increasing thin-film friction can increase torque capacity in transmissions and reduce the tendency for shudder to occur. It is also known that different additives normally present in a lubricant composition form films of different thicknesses, which can have an effect on thin-film friction. Moreover, some additives have a narrow range of conditions wherein they provide increased friction properties to a lubricant composition.

However, it is also known that some additives are very expensive. And, the use of additional amounts of an additive to a lubricant composition to increase thin-film friction can be quite costly to the manufacturer.

A major component of a lubricant composition can be the base oil, which is relatively inexpensive. Base oils are known and have been categorized under Groups I-V. The base oils are placed in a given Group based upon their % saturates, % sulfur content, and viscosity index. For example, all Group II base oils have greater than 90% saturates, less than 0.03% sulfur, and a viscosity index ranging from  $\geq 80$  to  $\leq 120$ . However, the proportions of aromatics, paraffinics, and naphthenics can vary substantially in the Group II base oils. It is known that the difference in these proportions can affect the properties of a lubricant composition, such as oxidative stability.

What is needed is a lubricant composition that is inexpensive and can provide at least one of increased thin-film friction and increased torque capacity or decreased tendency for shudder.

## SUMMARY

In accordance with the disclosure, there is disclosed a lubricant composition comprising a dispersant and a base oil comprising more than about 1.6% by weight of tetracycloparaffins.

There is also disclosed method of increasing the thin-film friction of a fluid between surfaces comprising providing to the fluid a composition comprising a dispersant and a base oil comprising more than about 1.6% by weight of tetracycloparaffins.

In an aspect, there is disclosed a method of increasing torque capacity in a transmission comprising providing to a transmission a composition comprising a dispersant and a base oil comprising more than about 1.6% by weight of tetracycloparaffins.

## 2

Further, there is disclosed a method of making a lubricant composition comprising combining a dispersant and a base oil comprising more than about 1.6% by weight of tetracycloparaffins.

Additional objects and advantages of the disclosure will be set forth in part in the description which follows, or may be learned by practice of the invention. The objects and advantages of the disclosure will be realized and attained by means of the elements and combinations particularly pointed out in the appended claims.

It is to be understood that both the foregoing general description and the following detailed description are exemplary and explanatory only and are not restrictive of the disclosure, as claimed.

## DESCRIPTION OF THE EMBODIMENTS

The present disclosure relates to lubricating compositions comprising a base oil comprising more than about 1.6% by weight of tetracycloparaffins and a dispersant. The base oil can be any base oil categorized in Groups I-V. In an aspect, the base oil is a Group II base oil. The base oil can comprise more than about 1.6% by weight, for example more than about 2% by weight, and as a further example more than about 3% by weight of tetracycloparaffins relative to the total weight of the base oil.

The disclosed base oils can have a higher thin-film friction coefficient as compared to base oils not comprising more than about 1.6% by weight of tetracycloparaffins. Moreover, it is believed, without being limited to any particular theory, that when the concentration of base oil structures is increased the effect of individual additives on thin-film friction is altered. In an aspect, the combination of certain additives with the disclosed base oil can have a synergistic effect.

The base oil can be present in the lubricating composition in any desired or effective amount. For example, the base oil can be present in a major amount. A "major amount" is understood to mean greater than or equal to 50% by weight relative to the total weight of the composition. As a further example, the base oil can be present in an amount greater than or equal to 80%, and as an additional example, greater than or equal to 90% by weight relative to the total weight of the composition.

The dispersant for use in the disclosed lubricating composition can be selected from any of the ashless dispersants known to those skilled in the art. Suitable ashless dispersants may include ashless dispersants such as succinimide dispersants, Mannich base dispersants, and polymeric polyamine dispersants. Hydrocarbyl-substituted succinic acylating agents can be used to make hydrocarbyl-substituted succinimides. The hydrocarbyl-substituted succinic acylating agents include, but are not limited to, hydrocarbyl-substituted succinic acids, hydrocarbyl-substituted succinic anhydrides, the hydrocarbyl-substituted succinic acid halides (for example, the acid fluorides and acid chlorides), and the esters of the hydrocarbyl-substituted succinic acids and lower alcohols (e.g., those containing up to 7 carbon atoms), that is, hydrocarbyl-substituted compounds which can function as carboxylic acylating agents.

Hydrocarbyl substituted acylating agents can be made by reacting a polyolefin or chlorinated polyolefin of appropriate molecular weight with maleic anhydride. Similar carboxylic reactants can be used to make the acylating agents. Such reactants can include, but are not limited to, maleic acid, fumaric acid, malic acid, tartaric acid, itaconic acid, itaconic anhydride, citraconic acid, citraconic anhydride, mesaconic acid, ethylmaleic anhydride, dimethylmaleic anhydride, eth-

ylmaleic acid, dimethylmaleic acid, hexylmaleic acid, and the like, including the corresponding acid halides and lower aliphatic esters.

The molecular weight of the olefin can vary depending upon the intended use of the substituted succinic anhydrides. Typically, the substituted succinic anhydrides can have a hydrocarbyl group of from about 8-500 carbon atoms. However, substituted succinic anhydrides used to make lubricating oil dispersants can typically have a hydrocarbyl group of about 40-500 carbon atoms. With high molecular weight substituted succinic anhydrides, it is more accurate to refer to number average molecular weight ( $M_n$ ) since the olefins used to make these substituted succinic anhydrides can include a mixture of different molecular weight components resulting from the polymerization of low molecular weight olefin monomers such as ethylene, propylene and isobutylene.

The mole ratio of maleic anhydride to olefin can vary widely. It can vary, for example, from about 5:1 to about 1:5, or for example, from about 1:1 to about 3:1. With olefins such as polyisobutylene having a number average molecular weight of about 500 to about 7000, or as a further example, about 800 to about 3000 or higher and the ethylene-alpha-olefin copolymers, the maleic anhydride can be used in stoichiometric excess, e.g. 1.1 to 3 moles maleic anhydride per mole of olefin. The unreacted maleic anhydride can be vaporized from the resultant reaction mixture.

Polyalkenyl succinic anhydrides can be converted to polyalkyl succinic anhydrides by using conventional reducing conditions such as catalytic hydrogenation. For catalytic hydrogenation, a suitable catalyst is palladium on carbon. Likewise, polyalkenyl succinimides can be converted to polyalkyl succinimides using similar reducing conditions.

The polyalkyl or polyalkenyl substituent on the succinic anhydrides employed herein can be generally derived from polyolefins which are polymers or copolymers of mono-olefins, particularly 1-mono-olefins, such as ethylene, propylene and butylene. The mono-olefin employed can have about 2 to about 24 carbon atoms, or as a further example, about 3 to about 12 carbon atoms. Other suitable mono-olefins include propylene, butylene, particularly isobutylene, 1-octene and 1-decene. Polyolefins prepared from such mono-olefins include polypropylene, polybutene, polyisobutene, and the polyalphaolefins produced from 1-octene and 1-decene.

In some aspects, the ashless dispersant can include one or more alkenyl succinimides of an amine having at least one primary amino group capable of forming an imide group. The alkenyl succinimides can be formed by conventional methods such as by heating an alkenyl succinic anhydride, acid, acid-ester, acid halide, or lower alkyl ester with an amine containing at least one primary amino group. The alkenyl succinic anhydride can be made readily by heating a mixture of polyolefin and maleic anhydride to about 180°-220° C. The polyolefin can be a polymer or copolymer of a lower monoolefin such as ethylene, propylene, isobutene and the like, having a number average molecular weight in the range of about 300 to about 3000 as determined by gel permeation chromatography (GPC).

Amines which can be employed in forming the ashless dispersant include any that have at least one primary amino group which can react to form an imide group and at least one additional primary or secondary amino group and/or at least one hydroxyl group. A few representative examples are: N-methyl-propanediamine, N-dodecylpropanediamine, N-aminopropyl-piperazine, ethanolamine, N-ethanol-ethylenediamine, and the like.

Suitable amines can include alkylene polyamines, such as propylene diamine, dipropylene triamine, di-(1,2-butylene)

triamine, and tetra-(1,2-propylene)pentamine. A further example includes the ethylene polyamines which can be depicted by the formula  $H_2N(CH_2CH_2-NH)_nH$ , wherein n can be an integer from about one to about ten. These include: 5 ethylene diamine, diethylene triamine (DETA), triethylene tetramine (TETA), tetraethylene pentamine (TEPA), pentaethylene hexamine (PEHA), and the like, including mixtures thereof in which case n is the average value of the mixture. Such ethylene polyamines have a primary amine group at 10 each end so they can form mono-alkenylsuccinimides and bis-alkenylsuccinimides. Commercially available ethylene polyamine mixtures can contain minor amounts of branched species and cyclic species such as N-aminoethyl piperazine, 15 N,N'-bis(aminoethyl)piperazine, N,N'-bis(piperazinyl)ethane, and like compounds. The commercial mixtures can have approximate overall compositions falling in the range corresponding to diethylene triamine to tetraethylene pentamine. The molar ratio of polyalkenyl succinic anhydride to polyalkylene polyamines can be from about 1:1 to about 3.0:1. 20

In some aspects, the dispersant can include the products of the reaction of a polyethylene polyamine, e.g. triethylene tetramine or tetraethylene pentamine, with a hydrocarbon substituted carboxylic acid or anhydride made by reaction of 25 a polyolefin, such as polyisobutene, of suitable molecular weight, with an unsaturated polycarboxylic acid or anhydride, e.g., maleic anhydride, maleic acid, fumaric acid, or the like, including mixtures of two or more such substances.

Polyamines that are also suitable in preparing the dispersants described herein include N-arylphenylenediamines, such as N-phenylphenylenediamines, for example, N-phenyl-1,4-phenylenediamine, N-phenyl-1,3-phenylenediamine, and N-phenyl-1,2-phenylenediamine; aminothiazoles such as aminothiazole, aminobenzothiazole, aminobenzothiadiazole and aminoalkylthiazole; aminocarbazoles; aminoindoles; aminopyrroles; amino-indazolinones; aminomercaptotriazoles; aminoperimidines; aminoalkyl imidazoles, such as 1-(2-aminoethyl)imidazol-e, 1-(3-aminopropyl)imidazole; and aminoalkyl morpholines, such as 4-(3-aminopropyl)morpholine. These polyamines are described in more detail in U.S. Pat. Nos. 4,863,623 and 5,075,383, the disclosures of which are hereby incorporated by reference herein.

Additional polyamines useful in forming the hydrocarbyl-substituted succinimides include polyamines having at least one primary or secondary amino group and at least one tertiary amino group in the molecule as taught in U.S. Pat. Nos. 5,634,951 and 5,725,612, the disclosures of which are hereby incorporated by reference herein. Non-limiting examples of suitable polyamines include N,N,N',N"-tetraalkyldialkylbenzylamines (two terminal tertiary amino groups and one central secondary amino group), N,N,N',N"-tetraalkyltrialkylketenetetramines (one terminal tertiary amino group, two internal tertiary amino groups and one terminal primary amino group), N,N,N",N""-pentaalkyltrialkylketenetetramines (one terminal tertiary amino group, two internal tertiary amino groups and one terminal secondary amino group), tris(dialkylaminoalkyl)aminoalkylmethanes (three terminal tertiary amino groups and one terminal primary amino group), and like compounds, wherein the alkyl groups are the same or different and typically contain no more than about 12 carbon atoms each, and which can contain from about 1 to about 4 carbon atoms each. As a further example, these alkyl groups can be methyl and/or ethyl groups. Polyamine reactants of this type can include dimethylaminopropylamine (DMAPA) and N-methyl piperazine.

Hydroxyamines suitable for herein include compounds, oligomers or polymers containing at least one primary or

secondary amine capable of reacting with the hydrocarbyl-substituted succinic acid or anhydride. Examples of hydroxyamines suitable for use herein include aminoethyl-ethanolamine (AEEA), aminopropylmethanolamine (AP-DEA), ethanolamine, diethanolamine (DEA), partially propoxylated hexamethylene diamine (for example HMDA-2PO or HMDA-3PO), 3-amino-1,2-propanediol, tris(hydroxymethyl)aminomethane, and 2-amino-1,3-propanediol.

The mole ratio of amine to hydrocarbyl-substituted succinic acid or anhydride can range from about 1:1 to about 3:0.1. Another example of a mole ratio of amine to hydrocarbyl-substituted succinic acid or anhydride may range from about 1.5:1 to about 2.0:1.

The foregoing dispersant can also be a post-treated dispersant made, for example, by treating the dispersant with maleic anhydride and boric acid as described, for example, in U.S. Pat. No. 5,789,353, or by treating the dispersant with non-ylphenol, formaldehyde and glycolic acid as described, for example, in U.S. Pat. No. 5,137,980, the disclosures of which are hereby incorporated by reference in their entirety.

The Mannich base dispersants can be a reaction product of an alkyl phenol, typically having a long chain alkyl substituent on the ring, with one or more aliphatic aldehydes containing from about 1 to about 7 carbon atoms (for example, formaldehyde and derivatives thereof), and polyamines (especially polyalkylene polyamines). For example, a Mannich base ashless dispersants can be formed by condensing about one molar proportion of long chain hydrocarbon-substituted phenol with from about 1 to about 2.5 moles of formaldehyde and from about 0.5 to about 2 moles of polyalkylene polyamine.

Hydrocarbon sources for preparation of the Mannich polyamine dispersants can be those derived from substantially saturated petroleum fractions and olefin polymers, such as polymers of mono-olefins having from 2 to about 6 carbon atoms. The hydrocarbon source generally contains, for example, at least about 40 carbon atoms, and as a further example, at least about 50 carbon atoms to provide substantial oil solubility to the dispersant. The olefin polymers having a GPC number average molecular weight range from about 600 to 5,000 can be suitable. However, polymers of higher molecular weight can also be used. Suitable hydrocarbon sources can be isobutylene polymers and polymers made from a mixture of isobutene and a raffinate stream.

Suitable Mannich base dispersants can be Mannich base ashless dispersants formed by condensing about one molar proportion of long chain hydrocarbon-substituted phenol with from about 1 to about 2.5 moles of formaldehyde and from about 0.5 to about 2 moles of polyalkylene polyamine.

Polymeric polyamine dispersants suitable as the ashless dispersants are polymers containing basic amine groups and oil solubilizing groups (for example, pendant alkyl groups having at least about 8 carbon atoms). Such materials are illustrated by interpolymers formed from various monomers such as decyl methacrylate, vinyl decyl ether or relatively high molecular weight olefins, with aminoalkyl acrylates and aminoalkyl acrylamides. Examples of polymeric polyamine dispersants are set forth in U.S. Pat. Nos. 3,329,658; 3,449,250; 3,493,520; 3,519,565; 3,666,730; 3,687,849; and 3,702,300. Polymeric polyamines can include hydrocarbyl polyamines wherein the hydrocarbyl group is composed of the polymerization product of isobutene and a raffinate I stream as described above. PIB-amine and PIB-polyamines may also be used.

Methods for the production of ashless dispersants as described above are known to those skilled in the art and are reported in the patent literature. For example, the synthesis of

various ashless dispersants of the foregoing types is described in such patents as U.S. Pat. Nos. 2,459,112; 2,962,442, 2,984,550; 3,036,003; 3,163,603; 3,166,516; 3,172,892; 3,184,474; 3,202,678; 3,215,707; 3,216,936; 3,219,666; 3,236,770; 3,254,025; 3,271,310; 3,272,746; 3,275,554; 3,281,357; 3,306,908; 3,311,558; 3,316,177; 3,331,776; 3,340,281; 3,341,542; 3,346,493; 3,351,552; 3,355,270; 3,368,972; 3,381,022; 3,399,141; 3,413,347; 3,415,750; 3,433,744; 3,438,757; 3,442,808; 3,444,170; 3,448,047; 3,448,048; 3,448,049; 3,451,933; 3,454,497; 3,454,555; 3,454,607; 3,459,661; 3,461,172; 3,467,668; 3,493,520; 3,501,405; 3,522,179; 3,539,633; 3,541,012; 3,542,680; 3,543,678; 3,558,743; 3,565,804; 3,567,637; 3,574,101; 3,576,743; 3,586,629; 3,591,598; 3,600,372; 3,630,904; 3,632,510; 3,632,511; 3,634,515; 3,649,229; 3,697,428; 3,697,574; 3,703,536; 3,704,308; 3,725,277; 3,725,441; 3,725,480; 3,726,882; 3,736,357; 3,751,365; 3,756,953; 3,793,202; 3,798,165; 3,798,247; 3,803,039; 3,804,763; 3,836,471; 3,862,981; 3,872,019; 3,904,595; 3,936,480; 3,948,800; 3,950,341; 3,957,746; 3,957,854; 3,957,855; 3,980,569; 3,985,802; 3,991,098; 4,006,089; 4,011,380; 4,025,451; 4,058,468; 4,071,548; 4,083,699; 4,090,854; 4,173,540; 4,234,435; 4,354,950; 4,485,023; 5,137,980, and Re 26,433, herein incorporated by reference.

An example of a suitable ashless dispersant is a borated dispersant. Borated dispersants can be formed by boronating ("borating") an ashless dispersant having basic nitrogen and/or at least one hydroxyl group in the molecule, such as a succinimide dispersant, succinamide dispersant, succinic ester dispersant, succinic ester-amide dispersant, Mannich base dispersant, or hydrocarbyl amine or polyamine dispersant. Methods that can be used for borating the various types of ashless dispersants described above are described in U.S. Pat. Nos. 3,087,936; 3,254,025; 3,281,428; 3,282,955; 2,284,409; 2,284,410; 3,338,832; 3,344,069; 3,533,945; 3,658,836; 3,703,536; 3,718,663; 4,455,243; and 4,652,387, the disclosures of which are hereby incorporated by reference in their entirety.

The borated dispersant can include a high molecular weight dispersant treated with boron such that the borated dispersant includes up to about 2 wt % of boron, for example from about 0.8 wt % or less of boron, as a further example from about 0.1 to about 0.7 wt % of boron, as an even further example, from about 0.25 to about 0.7 wt % of boron, and as a further example from about 0.35 to about 0.7 wt % of boron. The dispersant can be dissolved in oil of suitable viscosity for ease of handling. It should be understood that the weight percentages given here are for neat dispersant, without any diluent oil added.

A dispersant can be further reacted with an organic acid, an anhydride, and/or an aldehyde/phenol mixture. Such a process can enhance compatibility with elastomer seals, for example. The borated dispersant can further include a mixture of borated dispersants. As a further example, the borated dispersant can include a nitrogen-containing dispersant and/or may be free of phosphorus.

A dispersant can be present in the lubricating composition in an amount of about 0.1 wt % to about 10 wt %, for example from about 1 wt % to about 7 wt %, and as a further example from about 2 wt % to about 5 wt % of the lubricating composition.

In an aspect, the dispersant for use in the disclosed lubricant composition can be an ethylene-propylene dispersant. In particular, the dispersant can be an ethylene-propylene copolymer grafted with maleic anhydride and reacted with n-phenyl phenylene diamine.

Low molecular weight ethylene-alpha-olefin succinic anhydride dispersants, as described in U.S. Pat. Nos. 5,075,383 and 6,117,825, the disclosures of which are hereby incorporated by reference, are also suitable for use herein. Also suitable in the present disclosure are ethylene alpha-olefin polymers as described in U.S. Pat. Nos. 5,266,223; 5,350,532; and 5,435,926, the disclosures of which are hereby incorporated by reference. Ethylene-propylene diene polymers, such as those described in U.S. Pat. Nos. 4,952,637, 5,356,999, 5,374,364, and 5,424,366, the disclosures of which are hereby incorporated by reference, are also suitable.

A cross-linked low molecular weight ethylene-propylene succinic anhydride dispersant is also suitable for use in the present invention. These cross-linked dispersants are similar to the low molecular weight ethylene alpha-olefin succinic anhydride dispersants discussed above, but additionally contain a multifunctional polyamine to achieve advantageous cross linking, as described in U.S. Pat. No. 6,107,258, the disclosure of which is hereby incorporated by reference.

Suitable dispersants will be derived from ethylene-alpha-olefin polymers having a molecular weight of ranging from about 300 to about 25,000, for example from about 1000 to about 15,000; more as a further example from about 5,000 to about 15,000.

In an additional aspect, the dispersant can be a highly grafted, amine derivatized functionalized ethylene-propylene copolymer as described fully in U.S. Pat. Nos. 5,139,688 and 6,107,257, the disclosures of which are hereby incorporated by reference.

In an aspect, the dispersant can be a functionalized olefin copolymer. The polymer or copolymer substrate can be prepared from ethylene and propylene or it can be prepared from ethylene and at least one higher olefin within the range of  $C_3$  to  $C_{23}$  alpha-olefins.

Non-limiting examples of polymers for use herein include copolymers of ethylene and at least one  $C_3$  to  $C_{23}$  alpha-olefins. In an aspect, copolymers of ethylene and propylene can be used. Other alpha-olefins suitable in place of propylene to form the copolymer or to be used in combination with ethylene and propylene to form a terpolymer include 1-butene, 2-butene, isobutene, 1-pentene, 1-hexene, 1-octene and styrene;  $\alpha, \omega$ -diolefins such as 1,5-hexadiene, 1,6-heptadiene, 1,7-octadiene; branched chain alpha-olefins such as 4-methylbutene-1,5-methylpentene-1, and 6-methylheptene-1; and mixtures thereof.

More complex polymer substrates, often designated as interpolymers, can be prepared using a third component. The third component generally used to prepare an interpolymer substrate can be a polyene monomer selected from non-conjugated dienes and trienes. The non-conjugated diene component can be one having from 5 to 14 carbon atoms in the chain. For example, the diene monomer can be characterized by the presence of a vinyl group in its structure and can include cyclic and bicyclo compounds. Representative dienes include 1,4-hexadiene, 1,4-cyclohexadiene, dicyclopentadiene, 5-ethylidene-2-norbornene, 5-methylene-2-norbornene, 1,5-heptadiene, and 1,6-octadiene. A mixture of more than one diene can be used in the preparation of the interpolymer. In an embodiment, a non-conjugated diene for preparing a terpolymer or interpolymer substrate can be 1,4-hexadiene.

The triene component can have at least two non-conjugated double bonds, and up to about 30 carbon atoms in the chain. Typical trienes useful in preparing the interpolymer of the invention can be 1-isopropylidene-3 $\alpha$ ,4,7,7 $\alpha$ -tetrahydroindene, 1-isopropylidenedicyclopentadiene, dihydro-isodicyclopentadiene, and 2-(2-methylene-4-methyl-3-pentenyl)(2.2.1) bicyclo-5-heptene.

Ethylene-propylene or higher alpha-olefin copolymers can comprise from about 15 to 80 mole percent ethylene and from about 85 to 20 mole percent  $C_3$  to  $C_{23}$  alpha-olefin with, for example, mole ratios from about 35 to 75 mole percent ethylene and from about 65 to 25 mole percent of a  $C_3$  to  $C_{23}$  alpha-olefin, with for example proportions being from 50 to 70 mole percent ethylene and 50 to 30 mole percent  $C_3$  to  $C_{23}$  alpha-olefin, and as a further example proportions being from 55 to 65 mole percent ethylene and 45 to 35 mole percent  $C_3$  to  $C_{23}$  alpha-olefin.

Terpolymer Variations of the foregoing polymers can comprise from about 0.1 to 10 mole percent of a non-conjugated diene or triene.

The terms polymer and copolymer can be used generically to encompass ethylene copolymers, terpolymers or interpolymers. These materials can comprise minor amounts of other olefinic monomers so long as the basic characteristics of the ethylene copolymers are not materially changed. One of ordinary skill in the art would understand how to make these functionalized olefin copolymers. For example, U.S. Pat. No. 6,107,257, the disclosure of which is hereby incorporated by reference, discloses methods for making functionalized olefin copolymers comprising units derived from: (A) about 12 to about 18 weight percent methyl methacrylate; (B) about 75 to about 85 weight percent of  $C_{10}$ - $C_{15}$  alkyl (meth)acrylate(s); and (C) about 2 to about 5 weight percent of a nitrogen-containing dispersant monomer. The polyalkyl (meth)acrylate copolymers can comprise the reaction products of: (A) from about 12 to about 18, weight percent methyl methacrylate; (B) from about 75 to about 85, weight percent of  $C_{10}$ - $C_{15}$  alkyl (meth)acrylate(s); and (C) from about 2 to about 5, weight percent of a nitrogen-containing dispersant monomer.

As used herein,  $C_{10}$ - $C_{15}$  alkyl (meth)acrylate means an alkyl ester of acrylic or methacrylic acid having a straight or branched alkyl group of 10 to 15 carbon atoms per group including, but not limited to, decyl (meth)acrylate, isodecyl (meth)acrylate, undecyl (meth)acrylate, lauryl (meth)acrylate, myristyl (meth)acrylate, dodecyl pentadecyl methacrylate, and mixtures thereof.

The alkyl (meth)acrylate comonomers containing 10 or more carbon atoms in the alkyl group can generally be prepared by standard esterification procedures using technical grades of long chain aliphatic alcohols, and these commercially available alcohols are mixtures of alcohols of varying chain lengths in the alkyl groups. Consequently, for the purposes of this disclosure, alkyl (meth)acrylate is intended to include not only the individual alkyl (meth)acrylate product named, but also to include mixtures of the alkyl (meth)acrylates with a predominant amount of the particular alkyl (meth)acrylate named.

The nitrogen-containing dispersant monomers suitable for use herein include dialkylamino alkyl (meth)acrylamides such as, N,N-dimethylaminopropyl methacrylamide; N,N-diethylaminopropyl methacrylamide; N,N-dimethylaminoethyl acrylamide and N,N-diethylaminoethyl acrylamide; and dialkylaminoalkyl (meth)acrylates such as N,N-dimethylaminoethyl methacrylate; N,N-diethylaminoethyl acrylate and N,N-dimethylaminoethyl thiomethacrylate.

In an aspect, the polyalkyl (meth)acrylate copolymers consist essentially of the reaction products of (A), (B) and (C). However, those skilled in the art will appreciate that minor levels of other monomers, polymerizable with monomers (A), (B) and/or (C) disclosed herein, can be present as long as they do not adversely affect the low temperature properties of the fully formulated fluids. Typically additional monomers are present in an amount of less than about 5 weight percent,

for example in an amount of less than 3 weight percent, and as a further example in an amount of less than 1 weight percent. For example, the addition of minor levels of monomers such as C<sub>2</sub>-C<sub>9</sub> alkyl (meth)acrylates, hydroxy- or alkoxy-containing alkyl (meth)acrylates, ethylene, propylene, styrene, vinyl acetate and the like are contemplated within the scope of this disclosure. In an aspect, the sum of the weight percent of (A), (B) and (C) equals 100%.

The copolymers can be prepared by various polymerization techniques including free-radical and anionic polymerization.

Conventional methods of free-radical polymerization can be used to prepare the copolymers. Polymerization of the acrylic and/or methacrylic monomers can take place under a variety of conditions, including bulk polymerization, solution polymerization, usually in an organic solvent, preferably mineral oil, emulsion polymerization, suspension polymerization and non-aqueous dispersion techniques.

Optionally, other components can be present in the lubricant composition. Non-limiting examples of other components include antiwear agents, detergent, diluents, defoamers, demulsifiers, anti-foam agents, corrosion inhibitors, extreme pressure agents, seal well agents, antioxidants, pour point depressants, rust inhibitors and friction modifiers.

The lubricating compositions disclosed herein can be used to lubricate anything. In an aspect, the lubricating composition can be an engine composition that is used to lubricate an engine. However, one of ordinary skill in the art would understand that the disclosed lubricating compositions can be used to lubricate anything, e.g., any surface, such as those where thin-film friction can be present. Moreover, there is disclosed a method of increasing thin-film friction of a fluid between surfaces comprising providing to the fluid the disclosed composition.

It is further envisioned that the lubricating compositions can be provided to any machinery wherein torque capacity is an issue. In particular, there is disclosed a method of increasing torque capacity in a transmission comprising providing to a transmission the disclosed composition.

Also disclosed herein is a method of lubricating a machine, such as an engine, transmission, automotive gear, a gear set, and/or an axle with the disclosed lubricating composition. In a further aspect, there is disclosed a method of improving fuel efficiency in a machine, such as an engine, transmission automotive gear, a gear set, and/or an axle comprising placing the disclosed lubricating composition in the machine, such as an engine, transmission, automotive gear, a gear set, and/or an axle.

## EXAMPLES

### Example 1

#### Base Oils

It is known in the industry that Group II base oils comprise more than 90% saturates, less than 0.03% sulfur, and have a viscosity index from about 80 to about 120. However, not all Group II base oils have the same thin-film frictional properties. The base oils in Table 1 were analyzed according to the procedure in Analytical Chemistry, 64:2227 (1992), the disclosure of which is hereby incorporated by reference, in order to determine the type of paraffins, cycloparaffins, and aromatics in the oil.

The thin-film friction coefficient of various known base oils (three Group II base oils and a PAO) was measured at 100° C./20N load with a 20% slide to roll ratio at 1.5 m/s.

TABLE 1

| Base Oils | Thin-Film Friction Coefficient | Kinematic Viscosity at 100° C. | % Tetracycloparaffins in Base Oil |
|-----------|--------------------------------|--------------------------------|-----------------------------------|
| A         | 0.066                          | 4.05 cSt                       | 3.33                              |
| B         | 0.030                          | 4.09 cSt                       | 1.57                              |
| PAO       | 0.027                          | 4.00 cSt                       | 0.00                              |

As shown in Table 1, a base oil A and a base oil B have similar kinematic viscosities, but base oil A has a higher thin-film friction coefficient. The results for PAO show that in an oil with no tetracycloparaffins thin-film friction is low.

Moreover, as shown in Table 1, the base oil having more than about 1.6% tetracycloparaffins exhibited a higher thin-film friction as compared to the other base oils. One of ordinary skill in the art would understand that the higher the thin-film friction the better the torque capacity.

### Example 2

#### Base Oils and Dispersants and Polymers

Various dispersants were mixed/blended/combined with each of base oil A and base oil C. The borated succinimide comprises about 0.072% by weight of boron. The thin-film friction coefficients were measured as described in Example 1. The results are shown in Table 2.

TABLE 2

|                                 | BASE OIL A | BASE OIL C |
|---------------------------------|------------|------------|
| +4% Succinimide                 | 0.082      | 0.029      |
| +4% Borated Succinimide         | 0.072      | 0.042      |
| +4% Mannich Dispersant          | 0.065      | 0.046      |
| +4% Low MW                      | 0.061      | 0.052      |
| functionalized olefin copolymer |            |            |
| +1% Olefin Copolymer            | 0.081      | 0.060      |
| +1% High MW                     | 0.068      | 0.047      |
| functionalized olefin copolymer |            |            |
| +1% Dispersant PMA              | 0.075      | 0.056      |

The results show that the thin-film friction coefficient is higher in all compositions comprising a base oil comprising less than about 1.6% by weight of tetracycloparaffins.

At numerous places throughout this specification, reference has been made to a number of U.S. patents, published foreign patent applications and published technical papers.

50 All such cited documents are expressly incorporated in full into this disclosure as if fully set forth herein.

For the purposes of this specification and appended claims, unless otherwise indicated, all numbers expressing quantities, percentages or proportions, and other numerical values 55 used in the specification and claims, are to be understood as being modified in all instances by the term "about." Accordingly, unless indicated to the contrary, the numerical parameters set forth in the following specification and attached claims are approximations that can vary depending upon the 60 desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques.

It is noted that, as used in this specification and the appended claims, the singular forms "a," "an," and "the,"

## 11

include plural referents unless expressly and unequivocally limited to one referent. Thus, for example, reference to "an antioxidant" includes two or more different antioxidants. As used herein, the term "include" and its grammatical variants are intended to be non-limiting, such that recitation of items in a list is not to the exclusion of other like items that can be substituted or added to the listed items.

While particular embodiments have been described, alternatives, modifications, variations, improvements, and substantial equivalents that are or can be presently unforeseen can arise to applicants or others skilled in the art. Accordingly, the appended claims as filed and as they can be amended are intended to embrace all such alternatives, modifications, variations, improvements, and substantial equivalents.

What is claimed is:

1. A lubricant composition comprising a dispersant and a base oil comprising more than about 1.6% by weight of tetracycloparaffins, wherein the dispersant is at least one of succinimide, borated succinimide, Mannich dispersant, functionalized olefin copolymer, and poly(meth)acrylate copolymer.

2. The composition of claim 1, wherein the dispersant is a succinimide.

3. The composition of claim 1, wherein the dispersant is a highly grafted, amine derivatized functionalized ethylene-propylene copolymer.

4. The composition of claim 1, wherein the dispersant is present in the lubricant composition in an amount ranging from about 0.1 wt. % to about 10 wt. % relative to the total weight of the composition.

5. The composition of claim 1, wherein the dispersant is present in the lubricant composition in an amount ranging from about 1 wt. % to about 7 wt. % relative to the total weight of the composition.

6. The composition of claim 1, further comprising antiwear agents, detergent, diluents, defoamers, demulsifiers, anti-foam agents, corrosion inhibitors, extreme pressure agents, seal well agents, antioxidants, pour point depressants, rust inhibitors and friction modifiers.

## 12

7. A method of increasing thin-film friction of a fluid between surfaces comprising providing to the fluid a composition comprising a dispersant and a base oil comprising more than about 1.6% by weight of tetracycloparaffins.

8. A method of increasing torque capacity in a transmission comprising providing to a transmission a composition comprising a dispersant and a base oil comprising more than about 1.6% by weight of tetracycloparaffins.

9. The method of claim 8, wherein the dispersant is at least one of succinimide, borated succinimide, Mannich dispersant, and functionalized olefin copolymer, poly(meth)acrylate copolymers.

10. The method of claim 9, wherein the dispersant is a succinimide.

11. The method of claim 8, wherein the dispersant is a highly grafted, amine derivatized functionalized ethylene-propylene copolymer.

12. The method of claim 8, wherein the dispersant is present in the lubricant composition in an amount ranging from about 0.1 wt. % to about 10 wt. % relative to the total weight of the composition.

13. A transmission lubricated with a lubricant composition according to claim 1.

14. A method of making a lubricant composition comprising combining a dispersant and a base oil comprising more than about 1.6% by weight of tetracycloparaffins.

15. The method of claim 14, wherein the dispersant is at least one of succinimide, borated succinimide, Mannich dispersant, and functionalized olefin copolymer, poly(meth)acrylate copolymers.

16. The method of claim 14, wherein the dispersant is present in the lubricant composition in an amount ranging from about 0.1 wt. % to about 10 wt. % relative to the total weight of the composition.

17. A method for lubricating a machine comprising providing to the machine the lubricant composition of claim 1.

18. The method of claim 17, wherein the machine is a transmission.

\* \* \* \* \*